# EUROPEAN PATENT SPECIFICATION

(11) **EP 2 649 169 B1**
(45) Date of publication and mention of the grant of the patent: **04.04.2018**
(21) Application number: 11796968.3
(22) Date of filing: 08.12.2011
(51) Int. Cl.: C10M 161/00, C10M 165/00

(54) **POLYMER THICKENED GREASE COMPOSITIONS WITH IMPROVED LOW FRICTION PROPERTIES**
MIT POLYMEREN VERDICKTE SCHMIERFETTZUSAMMENSETZUNGEN MIT VERBESSERTEN REIBUNGSARMEN EIGENSCHAFTEN
COMPOSITIONS DE GRAISSE ÉPAISSIES PAR POLYMÈRES PRÉSENTANT DES PROPRIÉTÉS SUPÉRIEURES EN TERMES DE FAIBLE COEFFICIENT DE FROTTEMENT

(30) Priority: 09.12.2010 WO PCT/EP2010/007486
(43) Date of publication of application: 16.10.2013
(73) Proprietor: Aktiebolaget SKF (publ), 415 50 Göteborg (SE)
(72) Inventor: PASARIBU, Rihard, NL-3439 MT Nieuwegein (NL); MEIJER, Dick, NL-3439 MT Nieuwegein (NL)
(74) Representative: Burö, Sven Peter
(86) International application number: PCT/EP2011/072163
(87) International publication number: WO 2012/076638

(56) References cited:
- EP-A1- 0 675 192
- EP-A2- 0 700 986
- WO-A1-2010/017909
- JP-A- 2005 112 955
- US-A1- 2003 069 147

## Description

### FIELD OF THE INVENTION

The present invention relates to a grease composition; a mechanical component onto which a layer of the grease composition has been applied; the use of the grease composition for bearing applications; the use of grease composition for reconditioning the lubrication of a mechanical component; the use of a polar wax in the preparation of a grease composition for bearing applications, the use of a polar wax in a grease composition for bearing applications; the use of the grease composition for reducing friction in a bearing, between bearing components or within a bearing application system; and a method for preparing the grease composition.

### BACKGROUND OF THE INVENTION

Polymer thickened lubricating greases and their preparation are known in the art. In US 3,392,119, a grease is described comprising a white mineral oil that has been thickened by means of a copolymer of ethylene and a homopolymer of polypropylene. In US 3,850,828, a lubricating grease composition has been described which is thickened with a polymeric mixture comprising a polyethylene and an atactic polypropylene. In EP 0700986 A2, a polymeric thickener for lubricating grease compositions is disclosed comprising containing a mixture of copolymers or homopolymers of polypropylene having a high molecular weight and a copolymer or homopolymer of propylene having a low molecular weight. Further, In EP 0942063, a lubricating grease composition is described comprising at least one polyolefin component, at least one base oil component and at least one rubber component.

These known polymer thickened lubricating grease compositions still leave room for improvement in respect of friction reduction in various bearing applications.

### SUMMARY OF THE INVENTION

Object of the present invention is to provide a new polymer thickened grease composition which displays an improved friction behaviour when compared to conventional grease compositions, including known polymer thickened grease compositions.

It has now been found that this can be established when a particular polymer thickened grease composition comprises a polar wax.

Accordingly, the present invention relates to a grease composition comprising:
(a) a lubricating base oil;
(b) a polymeric thickener comprising a mixture of (1) a (co- or homo)polymer of propylene with a weight average molecular weight of more than 200.000 and (2) a (co- or homo)polymer of propylene with a weight average molecular weight of less than 200.000; and
(c) a polar wax.

The present grease composition comprises:
(a) 60-95 wt% of the lubricating base oil;
(b) 1-20 wt% of the polymeric thickener; and
(c) 1-20 wt% of the polar wax, all weight percentages based on the total weight of the grease composition.

The present grease composition displays excellent low friction behaviour composition.

### DETAILED DESCRIPTION OF THE INVENTION

In the grease composition according to the present invention use is made of a polar wax. A polar wax is a wax which comprises a polar group in the wax components. Suitable polar waxes that can be used in accordance with the present invention include polyolefin waxes such as polar polypropylene wax , polar polyethylene wax, polar montan wax, polar derivatives of montan wax, such as esters, acids, fully saponified, partial saponified and emulisier containing esters. Preferably, the polar wax is a partially or fully saponified ester of a montanic acid, or an oxidized polyethylene wax. Montanic wax is obtainable from lignite or brown coal. Suitable waxes of a montanic acid derivative include esters of montanic acid. These montanic acid ester waxes may be partially or fully saponified. Specific examples of useful ester waxes from montanic acid to be used in accordance with the present invention include Licowax OM, Licowax OM FL and Licowax OP (as manufactured by Clariant Co.). Polar polyethylene waxes to be used in accordance with the present invention can suitably be prepared by oxidizing polyethylene wax or by oxidative decomposition of polymer grade polyethylene.

The polar polypropylene waxes to be used in accordance with the present invention can suitably be prepared by grafting polypropylene waxes with maleic anhydride.

Also, the grease composition according to the present invention comprises in addition a metal salt. The metal salt to be used in accordance with the present invention can be chosen from a wide variety of metals. Suitably, the metal of the metal salt is selected from the group consisting of Group 1A, 1B, 2A, 2B, 4A, 5A, 7B and 8B elements of the Periodic Table. Preferably, the metal in the metal salt is selected from the group consisting of bismuth, zinc, sodium, calcium, magnesium, antimony, barium, manganese, silver, gold, copper and lead. More preferably, the metal in the metal salt is bismuth, zinc or molybdenum. Even more preferably, the metal in the metal salt is bismuth or molybdenum. Most preferably, the metal in the metal salt is bismuth.

Suitably, the metal salt is selected from the group consisting of naphtenates, octoate, carbamate, carboxamides, sulfonamides, stearates, hydroxystearates and any mixture thereof. Preferably, the metal salt is a stearate, a hydroxystearate or a mixture thereof.

The polymer thickened grease to be used in accordance with the present invention comprises a polymeric thickener. In the present grease composition preferably only use is made of a polymeric thickener, not a conventional metal-based salt or metal-based soap thickener. However, a metal-based soap may be incorporated in the present grease composition as long as it does not adversely affect the overall properties of the grease composition.

It is observed that the metal salt to be used in accordance with the present invention does not act as a thickener. The metal salt to be used in accordance with the present invention is added to a grease composition that has already adequately been thickened by means of a polymer. The metal salt serves a different purpose, namely for lowering friction characteristics.

In case a metal salt is also present in the present grease composition, the grease composition suitably comprises:
(a) 60-95 wt% of the lubricating base oil;
(b) 1-20 wt% of the polymeric thickener; and
(c) 1-20 wt% of the polar wax,
(d) 1-20 wt% of the metal salt, all weight percentages based on the total weight of the grease composition.

The polymeric thickener to be used in the polymer thickened grease suitably comprises at least one component selected from the group consisting of natural rubber, synthetic rubber or rubber-like polymers, polypropylene, polyisoprene, polybutadiene, poly(styrenebutadiene), poly(ethylene-propylene-diene), polyurethane, polymethacrylate, polyisobutylene, poly(isobutylene-succinic acid), poly(isobutylene-succinic acid-polyacrylamide), polyurea and polyethylene.

The polymeric thickener to be used in accordance with the present invention comprises a first component and a second component, with the first component having a higher weight average molecular weight than the second component. The polymeric thickener comprises a high molecular weight component and a low molecular weight component, characterized in that the thickener comprises a mixture of (1) a (co- or homo-)polymer of propylene with a weight average molecular weight of more than 200.000 and (2) a (co- or homo-)polymer of propylene with a weight average molecular weight of less than 200.000.

Preferably, the polymeric thickener to be used in accordance with the present invention contains a high molecular weight component comprising a (co- or homo-)polymer of propylene with a weight average molecular weight in the range of from 200.000-350.000 and a low molecular weight component comprising a (co- or homo-) polymer of propylene with a weight average molecular weight in the range of from 20.000-200.000. Preferably, the low molecular weight component has a weight average molecular weight of less than 100.000, preferably in the range of from 50.000-100.000.

The weight ratio between the high molecular weight component and the low molecular weight component in the polymeric thickener can be in the range of from 1:40-3:1, suitably in the range of from 1:40-1:1, preferably in the range of from 1:40-1:5, more preferably in the range of from 1:25-1:15, and most preferably in the range of from 1:18-1:20. Outside this preferred range for the weight ratio between the high and low molecular weight components the final lubricating grease composition will generally not have desired application properties, in particular mechanical stability and consistency, i.e. be too "rubbery/elastic" and/or too "buttery". However, as the properties of the final composition are also dependent on the lubricant base oil and additives incorporated in grease compositions, as well as on the way the composition is prepared, other ratios may also be used for obtaining the desired properties of the final composition, as is well known to a man skilled in the art.

According to the present invention, the low molecular weight component is preferably a polypropylene homopolymer, more preferably a polypropylene homopolymer with a melt flow rate in the range of from of 500-1500 dg/min., especially in the range of from 750-1250 dg/min. as determined by test ASTM D 1238 L.

The high molecular weight component preferably has a melt flow rate (ASTM D-1238) in the range of from 1.5-15, more preferably in the range of from 1.5-7, most preferably in the range of from 3-5.
The low molecular weight component is preferably a polypropylene homopolymer.

Preferably, the high molecular weight component is a polypropylene homopolymer or a propylene/ethylene-copolymer.

The polymer thickener according to the invention is suitably used in the lubricating grease composition in an amount in the range of from 1-20, preferably in the range of from 5-15, more preferably in the range of from 8-12 percent by weight of the total grease composition. Other amounts can be used if desired.

Apart from the polymeric thickeners mentioned in detail hereinabove, the present grease composition may also contain other polymeric thickeners.

As the lubricating base oil any lubricating oil known per se may be used, such as mineral oils, synthetic hydrocarbons, ester oils, vegetable oils and mixtures thereof, of different viscosity. The type of base oil and viscosity can be selected to suit specific applications.

Furthermore, additives known per se may be incorporated in the lubricant grease composition, as long as they do not have a detrimental effect on the thickener composition, the base oil and/or the final grease composition. The grease composition may additionally comprise at least one additive component which is selected from the group consisting of antioxidants, corrosion inhibitors, anti-wear agents and pressure tolerance-increasing additives, and wherein the total content of the additive component(s) is in the range of from 0.2-15% by weight, and preferably in the range of from 1-8% by weight, based on the total weight of the grease composition.

In addition, the present invention relates to the use of a grease composition according to the present invention for bearing applications.

The present invention also relates to the use of the grease composition according to to the present invention for reducing friction in a bearing, between bearing components or within a bearing application system.

In addition, the present invention relates to a method for preparing a grease composition according to the present invention comprising the following steps:
a) mixing the polymeric thickener with the base lubricating oil at a temperature higher than the melting point of the polymers used; and
b) adding to the mixture obtained in step (a) the polar wax.

Suitably, during step (a) one or more anti-wear additives, anti-fretting additives, anticorrosion additives, anti-oxidants and/or other additives are additionally mixed with the other components. If a metal salt is also present in the present grease composition, the metal salt will usually be additionally mixed with other components in step (a).

Suitably, the wax and, if present, metal salt are heated prior to mixing. In this way an improved homogenising effect can be established. Preferably, a final mixing is carried out in step (a) using a three-roll mill or a ball-mill.

The polymeric thickener composition according to the invention can be prepared by mixing the polymers in a manner known per se, which can optionally involve heating. The polymers of the subject invention are mixed with a lubricating base oil and optional additives by means of conventional techniques known per se resulting in the grease composition according to the invention.

The preparation of the grease composition is preferably be carried out under a protective atmosphere, such as a nitrogen gas flow, for avoiding oxidation of the oils during heating.

According to a preferred embodiment the solid polymeric components and the lubricating base oil are heated together (preferably under stirring) to a temperature above the melting point of polypropylene, preferably in the range of from 190-210 °C, although other temperatures may be used if required.

After the polymers are dissolved in the lubricating base oil and optionally additives have been added, the grease is cooled from the mixing temperature to room temperature.

According to an especially preferred embodiment of the invention this cooling is carried out in a period of time in the range of from 1 sec.-3 min., preferably in the range of from 10 sec.-1 min., more preferably in the range of from 25-35 sec. This rapid cooling process, which forms an important aspect of the invention, will be indicated hereinbelow as "quenching". The quenching of the lubricant grease composition can be carried out, for instance, by pouring the grease composition on a metal plate, although any other suitable rapid cooling method may also be used, such as spraying.

The quenching process according to the invention has a major influence on the grease structure, giving significant improvement of the properties of the final grease compositions compared to both conventional lubricating greases, as well as lubricating greases according to the invention which are cooled slowly, e.g. in approximately 1 degree per minute by the use of conventional cooling methods, such as simply keeping the grease in the reaction vessel with external/internal cooling. This results, for the polymer grease, in a lubricant lacking any mechanical stability.

In the grease composition according to the invention, the polymeric thickener forms a sponge-like structure, which gives the grease its appearance and structure. The lubricating base oil is kept within the pore-like spaces within the thickener structure, and bleeds out during service of the grease. The thickener-structure is very irregular with large pores as well as very small pores. The above indicated quenching of the lubricant grease composition provides a grease according to the invention with a smoother and more uniform structure of the polymeric thickener, with more uniformly distributed spaces for keeping the lubricant oil.

During service of the lubricant grease, the oil bleeds out of the oil/thickener-structure onto the surfaces of the bearing, thereby providing the lubricating action. The oil bleeding characteristics at the service temperature of the lubricant grease composition (i.e. the running temperature of the bearing, as well as the "start up" temperature) are therefore critical for obtaining the lubricating action of the composition.

The mechanical stability of the grease is dependent on the polymer thickener used, the lubricating base oil used, as well as the additives used. Further, the mechanical properties of the grease can be influenced by "working" the grease after the thickener is mixed with the lubricating base oil, as is well known to a man skilled in the art of lubricants. Preferably, the grease is "worked" to a consistency desired and/or required for its intended use.

The mechanical stability of the grease can be ascertained by means of tests known in the art, such as the Shell roll stability test. Preferably, the grease will have a penetration after the Shell roll stability test (24 hrs at 80 °C, 165 rpm), of max. 360.

The consistency of the grease can be classified by means of the NLGI-class. According to the present invention the grease can usually be prepared to a NLGI-class range 0 to 4. Also, the viscosity of the separated oil must be acceptable, and preferably be constant.

The polymer-thickened grease composition according to the present invention can be used for all conventional applications for lubricant grease compositions, so long as these are compatible with the components of the lubricant grease composition. The present grease composition can be used for lubricating bearings, couplings, toothed transmission gears, chutes or other instruments.

The mechanical component having a metal surface to be treated with the grease composition according to the present invention is preferably a bearing, bearing component or a bearing application system. The bearing component may be inner rings, outer rings, cages, rollers, balls and seal-counter faces. The bearing application system in accordance with the present invention comprises bearing housings, mounting axles, shafts, bearing joints and shields.

The present invention further relates to a grease composition obtainable according to the method of the invention.

The grease composition in accordance with the present invention may have the form of a lubricant composition having an oily character or a paste, depending on the viscosity of the final grease composition.

The invention will now be further illustrated by the following Examples, which do not limit the invention in any way.

### Examples

### Example 1

A number of greases were used in a reciprocating sliding test. The grease compositions used in these test experiments are shown in Table 1. The reciprocating sliding test was carried out under the following conditions:
Configuration: hardened steel ball on hardened steel flat surface
Roughness of the ball (Ra): 10 nm
Roughness of flat surface (RA): 20 nm
Ball diameter: 6 mm
Normal load: 3.5 N (1 GPa Hertzian pressure)
Temperature: 60 °C
Stroke: 4 mm, 0.5 Hz

The results of these tests experiments in terms of coefficients of friction are shown in Table 2. From the test results shown in Table 2 it is evident that experiment No 1 wherein use of the grease composition according to the present invention shows a considerably improved low friction performance when compared with experiments 2-5 wherein use is made of conventional greases.

**Table 1**

| Grease composition | Composition of grease |
|---|---|
| Grease No. 1* | 11% polypropylene, 84% PAO base lubricating oil, 5% wax of partially saponified ester of montanic acid (Clariant - Licowax OMFL) |
| Grease No. 2* | 11% polypropylene, 89% PAO base lubricating oil |
| Grease No. 3** | SKF GHG (metal-based soap thickener in a mineral base oil) |
| Grease No. 4** | Kyodo Yushi, Raremax AF-1 (polyurea thickener in a mineral base oil) |
| Grease No. 5** | ESSO/Mobil, Infinitec 152 (metal-based soap thickener in poly alpha olefm base (PAO) oil) |

| | |
|---|---|
| * PAO (poly alpha olefin) ** commercially available grease | |

**Table 2**

| Experiment No. | Grease composition | Coefficient of Friction |
|---|---|---|
| Experiment No. 1 | Grease No. 1 | 0.055 |
| Experiment No. 2 | Grease No. 2 | 0.08 |
| Experiment No. 3 | Grease No. 3 | 0.1 |
| Experiment No. 4 | Grease No. 4 | 0.09 |
| Experiment No. 5 | Grease No. 5 | 0.11 |

### Example 2

In this example greases Nos. 1-5 were subjected to a ball-on-disk test which was carried out under the following conditions.
Load: 300 N (1.9 GPa Hertzian pressure)
Disk: 100Cr6 cicrular ground; Ra 0.1 µm; Rq 0.14 µm
Ball: RB 20.638 G10
Slide to roll ratio: 5%
Constant entrainment speed: 0.05 m/s; 1.0 m/s.
Temperature: 40 °

The test results are shown in Table 3. From Table 3 it is clear that experiment No. 6 wherein use is made of a grease in accordance with the present invention displays a significantly improved low friction behaviour when compared with experiments 7-10 wherein use is made of conventional greases.

**Table 3**

| Experiment No. | Grease composition | Coefficient of Friction (constant entrainment speed 0.05 m/s) | Coefficient of Friction (constant entrainment speed 1.0 m/s) |
|---|---|---|---|
| Experiment No. 6 | Grease No. 1 | 0.03 | 0.035 |
| Experiment No. 7 | Grease No. 2 | 0.07 | 0.06 |
| Experiment No. 8 | Grease No. 3 | 0.055 | 0.07 |
| Experiment No. 9 | Grease No. 4 | 0.065 | 0.075 |
| Experiment No. 10 | Grease No. 5 | 0.06 | 0.07 |

### Example 3

A number of greases were used in a reciprocating sliding test. The grease compositions used in these test experiments are shown in Table 4. The reciprocating sliding test was carried out under the following conditions:
Configuration: hardened steel ball on flat surface polyoxymethylene surface
Roughness of the ball (Ra): 10 nm
Roughness of flat surface (RA): 20 nm
Ball diameter: 6 mm
Normal load: 3.4 N (1 GPa Hertzian pressure)
Temperature: 60 °C
Stroke: 4 mm, 0.5 Hz

The results of these tests experiments in terms of coefficients of friction are shown in Table 5. From the test results shown in Table 5 it is evident that experiment Nos. 11 and 12 wherein use of the grease composition according to the present invention show a considerably improved low friction performance when compared with experiment No. 13 wherein use is made of conventional grease.

**Table 4**

| Grease composition | Composition of grease |
|---|---|
| Grease No. 11* | 11% polypropylene, 79% PAO base lubricating oil, 5% wax of partially saponified ester of montanic acid (Clariant - Licowax OMFL), 5 % bismuth hydroxystearate |
| Grease No. 12* | 6% polypropylene, 74% PAO base lubricating oil, 5% oxidized polyethylene was (Licowax PED 121), 5% wax of partially saponified ester of montanic acid (Clariant - Licowax OMFL), 5% bismuth hydroxylstearate |
| Grease No. 13* | 11% polypropylene, 89% PAO base lubricating oil |

| | |
|---|---|
| * PAO (poly alpha olefin) | |

**Table 5**

| Experiment No. | Grease composition | Coefficient of Friction | Friction reduction (%) when compared to Exp. No. 13 |
|---|---|---|---|
| Experiment No. 11 | Grease No. 11 | 0.022 | 35 |
| Experiment No. 12 | Grease No. 12 | 0.015 | 55 |
| Experiment No. 13 | Grease No. 13 | 0.034 | - |

### Example 4

A number of greases were used in a reciprocating sliding test. The grease compositions used in these test experiments are shown in Table 6. The reciprocating sliding test was carried out under the following conditions:
Configuration: hardened steel ball on on hardened steel flat surface
Roughness of the ball (Ra): 10 nm
Roughness of flat surface (RA): 20 nm
Ball diameter: 6 mm
Normal load: 3.4 N (1 GPa Hertzian pressure)
Temperature: 60 °C
Stroke: 4 mm, 0.5 Hz

The results of these tests experiments in terms of coefficients of friction are shown in Table 7. From the test results shown in Table 5 it is evident that experiment No. 14-17 wherein use of the grease composition according to the present invention show a considerably improved low friction performance when compared with experiment No. 18 wherein use is made of conventional grease.

**Table 6**

| Grease composition | Composition of grease |
|---|---|
| Grease No. 14* | 11% polypropylene, 84% PAO base lubricating oil, 5% wax of partially saponified ester of montanic acid (Clariant - Licowax OMFL) |
| Grease No. 15* | 11% polypropylene, 84% PAO base lubricating oil, 5 % bismuth hydroxystearate |
| Grease No. 16* | 11% polypropylene, 79% PAO base lubricating oil, 10% oxidized polyethylene wax (Licowax PED 121) |
| Grease No. 17* | 11% polypropylene, 79% PAO base lubricating oil, 5% wax of partially saponified ester of montanic acid (Clariant - Licowax OMFL), 5% bismuth hydroxystearate |
| Grease No. 18* | 11% polypropylene, 89% PAO base lubricating |

| | |
|---|---|
| * PAO (poly alpha olefin) | |

**Table 7**

| Experiment No. | Grease composition | Coefficient of Friction | Friction reduction (%) when compared to Exp. No. 18 |
|---|---|---|---|
| Experiment No. 14 | Grease No. 14 | 0.053 | 29 |
| Experiment No. 15 | Grease No. 15 | 0.058 | 23 |
| Experiment No. 16 | Grease No. 16 | 0.055 | 27 |
| Experiment No. 17 | Grease No. 17 | 0.052 | 31 |
| Experiment No. 18 | Grease No. 18 | 0.075 | - |

## Claims

1. A grease composition comprising:
(a) 60-95 wt% of a lubricating base oil;
(b) 1-20 wt% of a polymeric thickener, the polymeric thickener comprising a mixture of (1) a (co- or homo)polymer of propylene with a weight average molecular weight of more than 200.000 and (2) a (co- or homo)polymer of propylene with a weight average molecular weight of less than 200.000; and
(c) 1-20 wt% of a polar wax, being a polar polypropylene wax, a polar polyethylene wax, a polar montan wax or a polar derivative of a montan wax, all weight percentages based on the total weight of the grease composition.

2. The grease composition according to claim 1, wherein the weight ratio between the high molecular weight component and the low molecular weight component is 1:40 - 1:5, preferably 1:25 - 1:15, more preferably 1:18-1:20.

3. The grease composition according to claim 2 or 3, wherein the low molecular weight component is a polypropylene homopolymer.

4. The grease composition according to any one of claims 1-3, wherein the low molecular weight component has a weight average molecular weight between 20.000 and 200.000 and a melt flow rate (ASTM D-1238) of 500-1500, preferably 750-1250.

5. The grease composition according to any of the claims 1-4, wherein the high molecular weight component is a polypropylene homopolymer or a propylene/ethylene-copolymer.

6. The grease composition according to any one of claims 1-5, wherein the high molecular weight component has a weight average molecular weight of 200.000-350.000 and a melt flow rate (ASTM D-1238) of 1.5-15, preferably 1.5-7.

7. The grease composition according to any one of claims 1-6 comprising in addition a metal salt which is selected from the group consisting of stearates, hydroxystearates and any mixture thereof.

8. The grease composition according to claim 7, wherein the metal of the metal salt is bismuth.

9. The grease composition according to any one of claims 1-8 which additionally comprises at least one additive component which is selected from the group consisting of antioxidants, corrosion inhibitors, anti-wear agents and pressure tolerance-increasing additives, and wherein the total content of the additive component(s) is in the range between 0.2 and 15% by weight, and preferably between 1 and 8% by weight, based on the total weight of the grease composition.

10. Use of a grease composition according to any one of claims 1-9 for bearing applications.

11. Use of a grease composition according to any one of claims 1-9 for reducing friction in a bearing, between bearing components or within a bearing application system.

12. A method for preparing a grease composition according to any one of claims 1-9 comprising the following steps:
a) mixing the polymeric thickener with the base lubricating oil at a temperature higher than the melting point of the polymers used; and
b) adding to the mixture obtained in step (a) the polar wax.

## Patentansprüche

1. Schmierfettzusammensetzung, umfassend:
(a) 60 bis 95 Gew.% eines Schmierbasisöls;
(b) 1 bis 20 Gew.% eines polymeren Verdickungsmittels, wobei das polymere Verdickungsmittel eine Mischung aus (1) (Co- oder Homo)polymer von Propylen mit einem durchschnittlichen Molekulargewicht (Gewichtsmittel) von mehr als 200.000 und (2) (Co- oder Homo)polymer von Propylen mit einem durchschnittlichen Molekulargewicht (Gewichtsmittel) von weniger als 200.000 umfasst; und
(c) 1 bis 20 Gew.% eines polaren Wachses, das ein polares Polypropylenwachs, ein polares Polyethylenwachs, ein polares Montanwachs oder ein polares Derivat von Montanwachs ist,
wobei sich alle Gewichtsprozentsätze auf das Gesamtgewicht der Schmierfettzusammensetzung beziehen.

2. Schmierfettzusammensetzung nach Anspruch 1, wobei das Gewichtsverhältnis zwischen der Komponente mit hohem Molekulargewicht und der Komponente mit niedrigem Molekulargewicht 1:40 bis 1:5, vorzugsweise 1:25 bis 1:15, bevorzugter 1:18 bis 1:20 beträgt.

3. Schmierfettzusammensetzung nach Anspruch 2 oder 3, wobei die Komponente mit niedrigem Molekulargewicht ein Polypropylenhomopolymer ist.

4. Schmierfettzusammensetzung nach einem der Ansprüche 1 bis 3, wobei die Komponente mit niedrigem Molekulargewicht ein durchschnittliches Molekulargewicht (Gewichtsmittel) zwischen 20.000 und 200.000 und eine Schmelzflussrate (ASTM D-1238) von 500 bis 1500, vorzugsweise 750 bis 1250 aufweist.

5. Schmierfettzusammensetzung nach einem der Ansprüche 1 bis 4, wobei die Komponente mit hohem Molekulargewicht ein Polypropylenhomopolymer oder ein Propylen/Ethylen-Copolymer ist.

6. Schmierfettzusammensetzung nach einem der Ansprüche 1 bis 5, wobei die Komponente mit hohem Molekulargewicht ein durchschnittliches Molekulargewicht (Gewichtsmittel) von 200.000 bis 350.000 und eine Schmelzflussrate (ASTM D-1238) von 1,5 bis 15, vorzugsweise 1,5 bis 7 aufweist.

7. Schmierfettzusammensetzung nach einem der Ansprüche 1 bis 6, die zusätzlich ein Metallsalz umfasst, das ausgewählt ist aus der Gruppe bestehend aus Stearaten, Hydroxystearaten und jedweder Mischung davon.

8. Schmierfettzusammensetzung nach Anspruch 7, wobei das Metall des Metallsalzes Wismut ist.

9. Schmierfettzusammensetzung nach einem der Ansprüche 1 bis 8, die zusätzlich mindestens eine Additivkomponente umfasst, die ausgewählt ist aus der Gruppe bestehend aus Antioxidantien, Korrosionsschutzmitteln, Antiverschleißmitteln und Drucktoleranz erhöhenden Additiven, und wobei der Gesamtgehalt der Additivkomponente(n) im Bereich zwischen 0,2 und 15 Gew.% und vorzugsweise zwischen 1 und 8 Gew.% liegt, bezogen auf das Gesamtgewicht der Schmierfettzusammensetzung.

10. Verwendung einer Schmierfettzusammensetzung gemäß einem der Ansprüche 1 bis 9 für Lageranwendungen.

11. Verwendung einer Schmierfettzusammensetzung gemäß einem der Ansprüche 1 bis 9 zur Herabsetzung der Reibung in einem Lager, zwischen Lagerkomponenten oder innerhalb eines Lageranwendungssystems.

12. Verfahren zur Herstellung einer Schmierfettzusammensetzung gemäß einem der Ansprüche 1 bis 9, umfassend die folgenden Schritte:
a) Mischen des polymeren Verdickungsmittels mit dem Basisschmieröl bei einer Temperatur, die höher als der Schmelzpunkt der verwendeten Polymere ist; und
b) Hinzufügen des polaren Wachses zu der in Schritt (a) erhaltenen Mischung.

## Revendications

1. Composition de graisse comprenant :
(a) 60 à 95 % en poids d'une huile de base lubrifiante ;
(b) 1 à 20 % en poids d'un épaississant polymère, l'épaississant polymère comprenant un mélange de (1) un (co-ou homo)polymère de propylène ayant une masse moléculaire moyenne en poids supérieure à 200 000 et (2) un (co-ou homo)polymère de propylène ayant une masse moléculaire moyenne en poids inférieure à 200 000 ; et
(c) 1 à 20 % en poids d'une cire polaire, ladite cire polaire étant une cire de polypropylène polaire, une cire de polyéthylène polaire, une cire de lignite polaire ou un dérivé polaire d'une cire de lignite,
tous les pourcentages en poids étant exprimés relativement au poids total de la composition de graisse.

2. Composition de graisse selon la revendication 1, dans laquelle le rapport pondéral entre le constituant à masse moléculaire élevée et le constituant à faible masse moléculaire est de 1:40 à 1:5, préférablement de 1:25 à 1:15, plus préférablement de 1:18 à 1:20.

3. Composition de graisse selon la revendication 2 ou 3, dans laquelle le constituant à faible masse moléculaire est un homopolymère de polypropylène.

4. Composition de graisse selon l'une quelconque des revendications 1 à 3, dans laquelle le constituant à faible masse moléculaire a une masse moléculaire moyenne en poids de 20 000 à 200 000 et un indice d'écoulement à l'état fondu (ASTM D-1238) de 500 à 1 500, préférablement de 750 à 1 250.

5. Composition de graisse selon l'une quelconque des revendications 1 à 4, dans laquelle le constituant à masse moléculaire élevée est un homopolymère de polypropylène ou un copolymère de propylène/éthylène.

6. Composition de graisse selon l'une quelconque des revendications 1 à 5, dans laquelle le constituant à masse moléculaire élevée a une masse moléculaire moyenne en poids de 200 000 à 350 000 et un indice d'écoulement à l'état fondu (ASTM D-1238) de 1,5 à 15, préférablement de 1,5 à 7.

7. Composition de graisse selon l'une quelconque des revendications 1 à 6, comprenant en outre un sel métallique qui est sélectionné dans le groupe constitué des stéarates, des hydroxystéarates et de n'importe quel mélange de ceux-ci.

8. Composition de graisse selon la revendication 7, dans laquelle le métal du sel métallique est le bismuth.

9. Composition de graisse selon l'une quelconque des revendications 1 à 8, laquelle comprend en outre au moins un constituant additif qui est sélectionné dans le groupe constitué des antioxydants, des inhibiteurs de corrosion, des agents anti-usure et des additifs augmentant la tolérance à la pression, et dans laquelle la teneur totale en constituant (s) additif(s) est de 0,2 à 15 % en poids, et préférablement de 1 à 8 % en poids, relativement au poids total de la composition de graisse.

10. Utilisation d'une composition de graisse selon l'une quelconque des revendications 1 à 9 pour des applications dans le domaine des roulements.

11. Utilisation d'une composition de graisse selon l'une quelconque des revendications 1 à 9 pour réduire le frottement dans un roulement, entre des éléments d'un roulement ou dans un système comportant un ou plusieurs roulements.

12. Procédé de préparation d'une composition de graisse selon l'une quelconque des revendications 1 à 9, comprenant les étapes qui consistent à :
a) mélanger l'épaississant polymère avec l'huile lubrifiante de base à une température supérieure au point de fusion des polymères utilisés ; et
b) ajouter la cire polaire au mélange obtenu à l'étape (a).
